



US007882884B2

(12) **United States Patent**  
Beals et al.

(10) **Patent No.:** US 7,882,884 B2  
(45) **Date of Patent:** \*Feb. 8, 2011

(54) **METHOD FOR CASTING CORE REMOVAL**

(75) Inventors: **James T. Beals**, West Hartford, CT (US); **Gary M. Lomasney**, Glastonbury, CT (US); **Joseph J. Parkos, Jr.**, East Haddam, CT (US)

(73) Assignee: **United Technologies Corporation**, Hartford, CT (US)

(\*) Notice: Subject to any disclaimer, the term of this patent is extended or adjusted under 35 U.S.C. 154(b) by 798 days.

This patent is subject to a terminal disclaimer.

(21) Appl. No.: 11/770,071

(22) Filed: Jun. 28, 2007

(65) **Prior Publication Data**

US 2008/0011445 A1 Jan. 17, 2008

**Related U.S. Application Data**

(62) Division of application No. 11/261,164, filed on Oct. 27, 2005, now Pat. No. 7,243,700.

(51) **Int. Cl.**  
**B22D 29/00** (2006.01)

(52) **U.S. Cl.** ..... 164/132; 164/345

(58) **Field of Classification Search** ..... 164/132, 164/345

See application file for complete search history.

(56) **References Cited**

## U.S. PATENT DOCUMENTS

4,141,781 A 2/1979 Greskovich et al.

|                |         |                             |
|----------------|---------|-----------------------------|
| 4,287,932 A    | 9/1981  | Schneider                   |
| 4,440,729 A    | 4/1984  | Jonsson                     |
| 5,332,023 A    | 7/1994  | Mills                       |
| 5,822,853 A    | 10/1998 | Ritter et al.               |
| 5,915,452 A    | 6/1999  | Conroy et al.               |
| 6,241,000 B1   | 6/2001  | Conroy et al.               |
| 6,637,500 B2   | 10/2003 | Shah et al.                 |
| 6,739,380 B2   | 5/2004  | Schlienger et al.           |
| 7,240,718 B2 * | 7/2007  | Schmidt et al. .... 164/132 |
| 7,243,700 B2 * | 7/2007  | Beals et al. .... 164/132   |

## OTHER PUBLICATIONS

European Office Action for EP Patent Application No. 06255488.6, dated Sep. 16, 2010.

\* cited by examiner

*Primary Examiner*—Kevin P Kerns

(74) *Attorney, Agent, or Firm*—Bachman & LaPointe, P.C.

(57) **ABSTRACT**

To destructively remove a casting core from a cast part, the part is exposed to a combination of nitric acid and sulfuric acid. The combination may have, by volume, a nitric acid concentration of 4-20 times the sulfuric acid concentration. The combination may be an aqueous solution including, by volume, 40-60% nitric acid and 3-10% sulfuric acid. The method may remove a ceramic casting core and a refractory metal-based casting core. A first leaching step may remove a major portion of the ceramic casting core and may comprise alkaline leaching. A second leaching step may remove a major portion of the refractory metal-based casting core and may comprise acid leaching. The acid leaching may comprise the combination of nitric acid and sulfuric acid.

23 Claims, 2 Drawing Sheets





FIG.1



FIG.2



FIG.3

## METHOD FOR CASTING CORE REMOVAL

## CROSS-REFERENCE TO RELATED APPLICATION

This is a divisional application of Ser. No. 11/261,164, filed Oct. 27, 2005, now U.S. Pat. No. 7,243,700 and entitled REFRACTORY METAL CORE REMOVAL, now U.S. Pat. No. 7,243,700, the disclosure of which is incorporated by reference in its entirety herein as if set forth at length.

## BACKGROUND

The disclosure relates to investment casting. More particularly, the disclosure relates to the removal of metallic casting cores from cast parts.

Investment casting is commonly used in the aerospace industry. Various examples involve the casting of gas turbine engine parts. Exemplary parts include various blades, vanes, seals, and combustor panels. Many such parts are cast with cooling passageways. The passageways may be formed using sacrificial casting cores.

Exemplary cores include ceramic cores, refractory metal cores (RMCs), and combinations thereof. In exemplary combinations, the ceramic cores may form feed passageways whereas the RMCs may form cooling passageways extending from the feed passageways through walls of the associated part.

After the initial casting of the part (e.g., from a nickel- or cobalt-based superalloy), the casting shell and core(s) are destructively removed. Exemplary shell removal is principally mechanical. Exemplary core removal is principally chemical. For example, the cores may be removed by chemical leaching. Exemplary leaching involves use of an alkaline solution in an autoclave.

An alternative acid leaching technique using nitric and sulfuric acid was proposed in U.S. Pat. No. 6,637,500.

Especially where long and/or fine passageways are concerned, the leaching may be quite time-consuming. Problems faced in leaching include: minimizing adverse effects on the cast part; and effective leaching of both metallic and ceramic cores where a combination is used.

## SUMMARY

One aspect of the disclosure involves a combination of nitric acid and sulfuric acid used to destructively remove at least one casting core (e.g., a refractory metal casting core) from a cast part. The combination has, by volume, a nitric acid concentration of 4-20 times a sulfuric acid concentration.

Another aspect of the disclosure involves a combination of nitric acid and sulfuric acid used to destructively remove at least one casting core (e.g., a refractory metal casting core) from a cast part. The combination has, by volume, 40-60% nitric acid and 3-10% sulfuric acid.

Another aspect of the disclosure involves a combination of an alkaline leaching and an acid leaching to remove at least one casting core (e.g., a combination of ceramic and refractory metal casting cores) from a cast part.

The details of one or more embodiments are set forth in the accompanying drawings and the description below. Other features, objects, and advantages will be apparent from the description and drawings, and from the claims.

## BRIEF DESCRIPTION OF THE DRAWINGS

FIG. 1 is a flowchart of an investment casting process.

FIG. 2 is a flowchart of an exemplary decoring process within the process of FIG. 1.

FIG. 3 is a flowchart of an alternate decoring process.

Like reference numbers and designations in the various drawings indicate like elements.

## DETAILED DESCRIPTION

FIG. 1 shows an exemplary method 20 for forming an investment casting mold. Other methods are possible, including a variety of prior art methods and yet developed methods. One or more metallic core elements are formed 22 (e.g., of refractory metals such as molybdenum and niobium by stamping or otherwise cutting from sheet metal) and coated 24. Suitable coating materials include silica, alumina, zirconia, chromia, mullite and hafnia. Preferably, the coefficient of thermal expansion (CTE) of the refractory metal and the coating are similar. Coatings may be applied by any appropriate line of sight or non line of sight technique (e.g., chemical or physical vapor deposition (CVD, PVD) methods, plasma spray methods, electrophoresis, and sol gel methods). Individual layers may typically be 0.1 to 1 mil thick. Layers of Pt, other noble metals, Cr, Si, W, and/or Al, or other non metallic materials may be applied to the metallic core elements for oxidation protection in combination with a ceramic coating for protection from molten metal erosion and dissolution.

One or more ceramic cores may also be formed 26 (e.g., of or containing silica in a molding and firing process). One or more of the coated metallic core elements (hereafter refractory metal cores (RMCs)) are assembled 28 to one or more of the ceramic cores. The core assembly is then overmolded 30 with an easily sacrificed material such as a natural or synthetic wax (e.g., via placing the assembly in a mold and molding the wax around it). There may be multiple such assemblies involved in a given mold.

The overmolded core assembly (or group of assemblies) forms a casting pattern with an exterior shape largely corresponding to the exterior shape of the part to be cast. The pattern may then be assembled 32 to a shelling fixture (e.g., via wax welding between end plates of the fixture). The pattern may then be shelled 34 (e.g., via one or more stages of slurry dipping, slurry spraying, or the like). After the shell is built up, it may be dried 36. The drying provides the shell with at least sufficient strength or other physical integrity properties to permit subsequent processing. For example, the shell containing the invested core assembly may be disassembled 38 fully or partially from the shelling fixture and then transferred 40 to a dewaxer (e.g., a steam autoclave). In the dewaxer, a steam dewax process 42 removes a major portion of the wax leaving the core assembly secured within the shell. The shell and core assembly will largely form the ultimate mold. However, the dewax process typically leaves a wax or byproduct hydrocarbon residue on the shell interior and core assembly.

After the dewax, the shell is transferred 44 to a furnace (e.g., containing air or other oxidizing atmosphere) in which it is heated 46 to strengthen the shell and remove any remaining wax residue (e.g., by vaporization) and/or converting hydrocarbon residue to carbon. Oxygen in the atmosphere reacts with the carbon to form carbon dioxide. Removal of the carbon may reduce or eliminate the formation of detrimental carbides in the metal casting. Removing carbon may also

reducine the potential for clogging the vacuum pumps used in subsequent stages of operation.

The mold may be removed from the atmospheric furnace, allowed to cool, and inspected **48**. The mold may be seeded **50** by placing a metallic seed in the mold to establish the ultimate crystal structure of a directionally solidified (DS) casting or a single-crystal (SX) casting. Nevertheless the present teachings may be applied to other DS and SX casting techniques (e.g., wherein the shell geometry defines a grain selector) or to casting of other microstructures. The mold may be transferred **52** to a casting furnace (e.g., placed atop a chill plate in the furnace). The casting furnace may be pumped down to vacuum **54** or charged with a non-oxidizing atmosphere (e.g., inert gas) to prevent oxidation of the casting alloy. The casting furnace is heated **56** to preheat the mold. This preheating serves two purposes: to further harden and strengthen the shell; and to preheat the shell for the introduction of molten alloy to prevent thermal shock and premature solidification of the alloy.

After preheating and while still under vacuum conditions, the molten alloy is poured **58** into the mold and the mold is allowed to cool to solidify **60** the alloy (e.g., after withdrawal from the furnace hot zone). After solidification, the vacuum may be broken **62** and the chilled mold removed **64** from the casting furnace. The shell may be removed in a deshelling process **66** (e.g., mechanical breaking of the shell).

The core assembly is removed in a decoring process **68** to leave a cast article (e.g., a metallic precursor of the ultimate part). Inventive multi-stage decoring processes are described below. The cast article may be machined **70**, chemically and/or thermally treated **72** and coated **74** to form the ultimate part. Some or all of any machining or chemical or thermal treatment may be performed before the decoring.

The exact nature of an appropriate decoring process **68** will depend on several factors. These factors include: the particular material(s) of the RMC(s), including any coating; the particular material(s) of any ceramic core(s); the particular casting alloy; and the core geometries. The materials provide various issues of effectiveness and compatibility with various removal techniques. The geometry issues influence the accessibility and required exposures.

A first group of exemplary inventive processes involve use of an acid leaching mechanism preferentially to remove the RMC(s). For example, the acid leaching mechanism may remove a majority of the RMC(s) while leaving the ceramic core(s) essentially or largely intact. An alkaline leaching mechanism may be used to preferentially remove the ceramic core(s). More broadly, the acid leaching mechanism may remove a greater proportion of one or more first RMC(s) than of one or more other cores (e.g., different RMCs or ceramic core(s)) and may remove a majority of the first RMC(s) while only a minor portion of the other core(s). The alkaline leaching mechanism may be used to preferentially remove the other core(s).

FIG. 2 shows one such exemplary decoring process wherein a alkaline leaching process **100** precedes an acid leaching process **102**. An exemplary alkaline process includes placing the casting in an autoclave and immersing the casting in an alkaline solution (e.g., 22.5% potassium Hydroxide). The solution exposure may be at an elevated pressure (e.g., 0.5 (75)-1.37 (200) MPa(PSI) gage) and a moderately elevated temperature (e.g., 350° F. (177° C.), more broadly 150-400° C., for an exemplary twelve hours, more broadly 1-72 hours). The pressure may be cycled and/or the solution otherwise agitated to maintain exposure of the alkaline solution to the ceramic and evacuate reaction prod-

ucts. There also may be intermediate rinses (e.g., with water at atmospheric pressure) to help evacuate reaction products.

After an optional cleaning rinse **104** (possibly including multiple rinse cycles with conductivity or other tests to determine rinse completion), the exemplary acid leaching process **102** includes immersing **106** the casting in an acid solution (e.g., a combination solution discussed below). The exposure may be at an elevated temperature. An exemplary temperature is lower then that of the alkaline autoclave. An exemplary temperature range is from ambient/room temperature to 120° F. (49° C.), more broadly to 80° C. The solution may be agitated to maintain exposure of the acid solution to the RMC and evacuate reaction products. Similarly, intermediate rinses **108** may aid evacuation and facilitate intermediate inspection **110**.

FIG. 3 shows another such exemplary decoring process wherein an acid leaching process **200** (e.g., similar to **102**) precedes an alkaline leaching process **202** (e.g., similar to **100**). This may be warranted where alkaline attack on the casting is sought to be minimized. Depending on core configuration, there may be a moderate increase in the time required for the acid leaching process (e.g., a doubling or slightly greater) relative to the FIG. 2 process. However, the alkaline leaching process may be reduced even more substantially (e.g., to less than a third). For example, access through outlet passageways left by an RMC may allow near instant attack by the alkaline solution along the length of a ceramic feedcore.

Experiments regarding the removal of molybdenum have indicated a number of relevant physical and chemical mechanisms for consideration in the selection of appropriate parameters of the acid leaching process. Nickel and cobalt superalloys in the cast, single crystal, and directionally solidified conditions were exposed to the combination of acids at varying temperatures from an ambient 70° F. (21° C.) to an elevated 150° F. (66° C.) for 24 hours. There were no adverse effects (<0.0005 inch material loss) on the tested alloys up to 120° F. (49° C.). Higher temperature yielded faster dissolution of the molybdenum RMC. Moderate etching of the casting was found at 150° F. (66° C.). Thus one recommended temperature for core removal without detrimental affects on the base material is near 120° F. (49° C.) (e.g., 100-140° F. (38-60° C.)).

Speed of removal from the casting is influenced by the accessibility of the RMC to the acid. Total dissolved metal also affects the dissolution rate. The rate drops rapidly when the total dissolved molybdenum exceeds 20 g/L. The solution ceases to perform satisfactorily beyond 30 g/L. Various combinations of concentrations of nitric acid and sulfuric acid were evaluated. A concentration of 50% nitric and 5% sulfuric provided good results balancing speed of removal and effect on the base metal. Agitation improved the rate by delivering fresh acid to the desired area but was thus not quantified.

From these experiments, it is seen that a synergistic combination of nitric acid (HNO<sub>3</sub>) and sulfuric acid (H<sub>2</sub>SO<sub>4</sub>) was discovered. An aqueous solution consisting essentially of, by volume, 40-60% nitric acid and 3-10% sulfuric acid would be expected to provide good results. For this solution, by volume, the nitric acid concentration may be an exemplary 4-20 times the sulfuric acid concentration, more narrowly 8-15 times.

One or more embodiments have been described. Nevertheless, it will be understood that various modifications may be made. For example, the principles may be implemented as modifications of existing or yet-developed processes in which cases those processes would influence or dictate parameters

## 5

of the implementation. Accordingly, other embodiments are within the scope of the following claims.

What is claimed is:

1. A method comprising:  
destructively removing a refractory metal-based casting core from a cast part by exposing the casting core to a combination of nitric acid and sulfuric acid, the combination having, by volume, a nitric acid concentration of 4-20 times a sulfuric acid concentration. 5
2. The method of claim 1 further comprising:  
molding a sacrificial pattern over said casting core; forming a shell over the pattern;  
destructively removing the pattern from the shell, leaving the casting core; 10  
casting a metallic material in the shell; and  
destructively removing the shell to leave the cast part. 15
3. The method of claim 1 wherein:  
the exposing is at a temperature of up to 80° C. 20
4. The method of claim 1 wherein:  
the casting core consists essentially of a refractory metal-based substrate, optionally coated. 20
5. The method of claim 4 wherein:  
the casting core is a first casting core; and  
the method includes removing a ceramic second casting core from the cast part, principally by alkaline leaching. 25
6. The method of claim 5 wherein:  
the alkaline leaching is substantially performed after the removal of the first casting core. 30
7. The method of claim 5 wherein:  
the alkaline leaching is substantially performed before the removal of the first casting core. 30
8. The method of claim 1 wherein the casting core consists essentially of a ceramic-coated molybdenum-based substrate. 35
9. The method of claim 1 wherein:  
the combination has a by volume nitric acid concentration of 8-15 times a sulfuric acid concentration. 35
10. The method of claim 1 wherein:  
the combination is in an aqueous solution including, by volume, 40-60% nitric acid and 3-10% sulfuric acid. 40
11. The method of claim 1 used to manufacture a gas turbine engine component. 40
12. The method of claim 1 wherein the cast part consists essentially of a nickel- or cobalt-based superalloy. 45
13. A method for removing a ceramic first casting core and a refractory metal-based second casting core from a cast part comprising:  
a first leaching step for removing a major portion of the first casting core and comprising alkaline leaching; and  
a second leaching step for removing a major portion of the second casting core and comprising acid leaching. 6
14. The method of claim 13 wherein:  
the first leaching step includes a plurality of first intervals at a pressure of 0.5 MPa to 1.37 MPa interposed with a plurality of second intervals at ambient pressure; and  
the second leaching step includes an interval at a temperature of 38-49° C. 10
15. The method of claim 13 wherein:  
the first leaching step includes at least one interval at a pressure of 0.5 MPa to 1.37 MPa gage; and  
the second leaching step includes an interval at a temperature of 38-49° C. 15
16. The method of claim 13 wherein:  
the first leaching step includes at least one interval at a pressure of at least 0.5 MPa gage; and  
the second leaching step includes at least one interval at a temperature of 30-49° C. 20
17. The method of claim 13 wherein:  
the second leaching step includes immersing in a solution containing nitric acid and sulfuric acid. 25
18. The method of claim 13 wherein:  
the first leaching step comprises exposing to a temperature of at least 100° C.; and  
the second leaching step comprises exposing to a temperature of up to 66° C. 30
19. The method of claim 13 wherein:  
the first leaching step comprises exposing to a temperature of at least 150° C.; and  
the second leaching step comprises exposing to a temperature of up to 60° C. 35
20. The method of claim 13 used to manufacture a gas turbine engine component. 35
21. The method of claim 13 wherein the cast part consists essentially of a nickel- or cobalt-based superalloy. 40
22. The method of claim 13 wherein the second core consists essentially of a ceramic-coated molybdenum-based substrate. 45
23. A method comprising:  
destructively removing a refractory metal-based casting core from a cast part by exposing the casting core to a combination of nitric acid and sulfuric acid, the combination being in an aqueous solution including, by volume, 40-60% nitric acid and 3-10% sulfuric acid. 45

## 6

\* \* \* \* \*